

May 26, 1936.

T. C. BROWNE

2,041,743

PRINTING PLATE MATRIX

Filed May 7, 1934



FIG. 1



FIG 2



FIG. 3



FIG. 4

FIG. 5



INVENTOR

Theodore C. Browne

BY  
Clyde A. Kotter  
ATTORNEY

## UNITED STATES PATENT OFFICE

2,041,743

## PRINTING PLATE MATRIX

Theodore C. Browne, Hinsdale, Ill.

Application May 7, 1934, Serial No. 724,273

5 Claims. (Cl. 41—25)

This invention relates to the graphic arts and is particularly directed to the production of a matrix in which resinous or resin-like running plates may be molded.

In my copending application Serial No. 670,238, filed May 10, 1933, I showed how resinous bodies might be cured under considerable pressure and formed into hard, dense masses conforming exactly to the original shape of the mold, even if the mold or matrix, as it is commonly called in the graphic arts, be of a soft, yielding nature.

In an application of Gilbert C. Waters, Serial No. 724,280, filed May 7, 1934, entitled Art of producing printing plates and matrices, a type or type-containing matrix was disclosed which because it is yieldable, extensible, but self-restoring, always can be removed from the type form no matter how broken the composition or deep the spaces between the type. It has the further advantages not found in previous matrices that the full shoulder depth of the type is always reproduced, that no surface grain or structure is introduced, and that shrinkage is practically eliminated. In fact, the shrinkage is so negligible that such a matrix retains multi-color registration in 133 line screen work perfectly.

This invention may be considered an improvement upon the processes set forth in the above applications and has for its objects to produce matrices from mixed forms containing a number of metals, to reduce the possibility of chemical damage to expensive half-tone originals; to prevent such chemical action as will render the production of a running plate in such a matrix difficult or impossible, and to produce matrices by "closed moulding".

Still other objects and advantages of my invention will be apparent from the specification.

The features of novelty which I believe to be characteristic of my invention are set forth with particularity in the appended claims. My invention itself, however, both as to its fundamental principles and as to its particular embodiments will best be understood by reference to the specification and accompanying drawing in which

Fig. 1 gives a perspective view of the form showing the chase modified according to my invention.

Fig. 2 is a transverse sectional view through the mould,

Fig. 3 is a sectional view of one form of matrix,

Fig. 4 is a similar section through an alternative form of matrix, and

Fig. 5 illustrates the method of manufacture, showing the press diagrammatically.

In the above identified Waters application the direction is given to plate the illustrations with some suitable metal such as tin, although nickel also is generally suitable.

Although the procedure outlined by Waters produces consistently excellent results when clean, fresh type metal makes up the form, it sometimes happens that the resin duplicates made in matrices formed on plated originals or electros, or from dirty, much-used type are full of minute blisters. In some cases, both the matrix and the resin running plate are full of small pits.

A chemical investigation of such matrices shows them to be poisoned with copper. From the exaggerated cases, intentionally produced in the experimental work on this invention I have found that copper-rubber, and particularly the copper-rubber-sulphur complexes, of whatever nature they may be, act like cement, in that they cause the sticking of resinous or resin-like masses to rubber. In some cases, it is impossible to separate the two without destroying either or both the plate and the matrix when the matrix bears even a very small amount of copper.

Sticking is not confined to one group of resins or even to resins, such very diverse chemical substances as phenol-formaldehyde resins, urea-formaldehyde resins, vinyl resins, chlorinated rubber, chlorinated rubber glucose mixtures, and the resin-like derivatives known as "plioform" stick violently, blister or form "fly-specks".

According to this invention, the working and entire resin-receiving surface of the matrix is made of sulphur-free material having rubber-like physical characteristics. If the matrix is to be made of rubber, tri-nitro-benzol instead of sulphur as taught by Ostromislensky in U. S. patents, 1,249,180, 1,249,181, and 1,646,409, is incorporated into the rubber as a vulcanizing agent. Successful matrices have been made containing—rubber 100 pts., 1, 3, 5 tri-nitro-benzol 2 pts., aniline, 1 pt., and carbon black 150 pts. which were cured 40 minutes in direct contact with copper, without any of the defects noted above.

I much prefer, because of greatly improved mechanical and surface characteristics obtainable, to make matrices having a working face of polymerized chloroprene, obtainable commercially under the name of "Duprene". Much information about this substance is available. It is well to point out, however, that its base substance bears such a resemblance to isoprene, the base substance of rubber, that great physical resemblance is to be expected.

5

10

15

20

25

30

35

40

45

50

55

5 Polymerized chloroprene cures in the presence of oxides and weak, organic acids, and more rapidly in the presence of organic acids and sulphur. For the present purpose, however, a composition 10 containing polymerized chloroprene, 400 pts.—, zinc oxide, 40 parts, magnesium oxide (light) 60 parts, "Lorol" 6 pts., wood resin 20 parts—, carbon black 160 parts—, mineral oil 12 parts, "Heliozone" 2 parts, cures sufficiently in ten minutes at eighty pounds gauge steam pressure and has no effect upon a fine-screen copper halftone. Neither does it pick up from the copper the extremely small amounts of "poison" which are sufficient to ruin a sulphur-bearing rubber matrix.

15 As the foregoing applications have pointed out, lateral deformation of the subsequent moldings or "pressings" is difficult to prevent in a rubber or rubber-like matrix, unless the rubber be cemented rigidly to a non-extensible member, preferably a thin sheet of spring brass.

20 Preferably also, the union of rubber to brass should occur as the matrix is being formed. Duprene will adhere to rubber when both are simultaneously cured and the rubber in turn will adhere to the prepared brass.

25 Although the open moulding procedure shown in the above identified applications is a great advantage where an enormous number of different sizes of forms are to be handled as in a jobbing electrotyper's establishment, it is not so certain as is closed moulding in producing a flat, fully filled matrix. It is possible to secure closed moulding advantages in establishments such as 30 book, magazine and catalog printing houses where a relatively few sizes of forms cover all needs by the following procedure.

35 The chase, 10, (Fig. 1) is of the ordinary cast iron or welded steel variety. It is surface ground to some convenient exact thickness and is provided with four locating holes 11, 11 drilled through the pads at the corners. The form is composed in the conventional manner except that wide, accurate type high steel bearers surround the composition and the "furniture" 13, is preferably of metal instead of wood. The form is held in place by the quoins 14.

40 I then provide a "nest" 15, which is an accurately ground plate of steel having a central moulding aperture 16. It carries four locating pins 17, 17 which engage the holes 11, 11. If the chase 10, is exactly type high (0.918") the shim 18 is unnecessary. Otherwise it is adjusted to bring the outside bearing for the nest exactly 45 type high. The plunger 19 is a flattened T having a leg or plunger portion 21 which fits within the aperture 16 with about .005" clearance, and a head 22.

50 In moulding the matrix, the chase 10 and the nest 15 are placed on the lower platen of a press 23, as shown in Fig. 5. A laminated sheet of gum stock having a polymerized chloroprene face and a backing layer of rubber gum stock is placed in the aperture 16. On this is placed a thin sheet of spring brass (covered with a cement to promote adhesion to the rubber) or a sheet of resin-cement covered resin-impregnated paper. Then the plunger 19 is put in place and the press closed against the top platen 24. Steam is admitted through the conduits 25, 25.

55 Under ordinary circumstances the inner face 26 of the head 22 engages the top surface 27 at the nest 15. The depth at the plunger section 21 controls the thickness at the matrix. If adjust-

ments of thickness are necessary, they may be made by interposing the bearers 28—28.

60 As the pressure is applied, the excess material is forced out over the gates 29, 29, cut in the bearers 12.

65 The necessary pressure and temperature are maintained until the cure is complete.

70 The time of cure is, of course, a function of the compounding. In the example given, the cure is complete in ten minutes at eighty pounds 10 steam.

75 I have found it advantageous to use as the backing layer a rubber compound which commercially is designated as "non-sulphur". The vulcanizing agent in this case is actually an organic sulphur compound which releases sulphur upon heating. So active, however, is the released sulphur that full cure is effected with as little as .017% combined sulphur.

80 With such a rubber, extremely thin layers of polymerized chloroprene are all that is necessary (a great advantage, since Duprene is as yet an expensive substance).

85 When ordinary sulphur rubber compounds are used (2½ to 3% sulphur) the excess sulphur is active and dangerous. Then thicker polymerized chloroprene is required to insulate and guard the copper from any possibility of sulphur attack.

90 The physical similarity of polymerized chloroprene to rubber is close. It is resilient, deformable, self-restoring after deformation, and produces a matrix which has many of the advantages of rubber. It may be pulled loose from any type form, however complicated, and restores itself so completely to the original size that registration of multicolor fine-screen, half-tone plates is easily secured.

95 A considerable number of rubber printing plates are now manufactured by moulding a thermo-setting resin matrix upon the type surface and thereafter moulding rubber therein. The mould herein described is adapted for the production of such matrices and I have produced extremely accurate and entirely satisfactory thermo-setting matrices therein.

100 While I have shown and described certain preferred embodiments of my invention, it will be understood that modifications and changes may be made without departing from the spirit and scope of my invention as will be evident to those skilled in the art.

I claim:

1. A matrix for the production of printing plates from molded plastics having an impression-bearing face comprising a layer of a sulphur-free resilient compound capable of relatively large deformation within its elastic limit, an intermediate layer of rubber, and a metallic back vulcanized and united together to form a unitary matrix element.

2. A flexible matrix comprising an impression-bearing face of a sulphur free chloroprene polymer, an intermediate layer of rubber and a reinforcing element which is substantially non-extensible under the pressures to which the matrix is designed to be subjected bonded together to form a single unitary structure.

3. A mold liner comprising an impression-bearing surface of a cured, flexible, yielding sulphur-free resilient substance capable of relatively large deformation within its elastic limit, an intermediate layer of vulcanized soft rubber and a reinforcing member.

4. A non-sticking mold liner for heat reactive

resin molding which comprises a resilient, yielding, surface of a substantially sulphur-free chloroprene polymer, a backing layer of rubber, and a reinforcing member having substantially zero lateral stretch.

5. A matrix for molding comprising an impres-

sion-bearing face of a sulphur-free resilient compound capable of relatively large deformation within its elastic limit, a layer of rubber containing substantially no uncombined sulphur, and a reinforcing backing member.

THEODORE C. BROWNE.